

United States Patent [19]  
Hiyama

[11] 3,876,512  
[45] Apr. 8, 1975

[54] ELECTROLYTIC CARBURIZING PROCESS  
USING A CARBONATE ELECTROLYTE

3,488,233 1/1970 Newell ..... 148/15.5  
3,635,768 1/1972 Mueller ..... 148/15.5

[75] Inventor: Shinji Hiyama, Kamakura-shi,  
Kanagawa, Japan

FOREIGN PATENTS OR APPLICATIONS  
155,812 7/1961 U.S.S.R. ..... 204/39

[73] Assignee: Nippon Furnace Koga Kaisha, Ltd.,  
Minatoku, Tokyo, Japan

Primary Examiner—R. L. Andrews  
Attorney, Agent, or Firm—John W. Logan, Jr., Esq.

[22] Filed: Sept. 10, 1973

[57] ABSTRACT

[21] Appl. No.: 395,541

A carburizing process consisting of using the object to be carburized as a cathode and inserting the cathode into an electrolytic bath including a melted metallic salt in which the anode is graphite.

[52] U.S. Cl. .... 204/39; 204/140

4 Claims, 2 Drawing Figures

[51] Int. Cl. .... C23b 11/00

[58] Field of Search ..... 204/39, 140; 148/15.5

[56] References Cited

UNITED STATES PATENTS

3,331,708 7/1967 Buitrus ..... 204/39



PATENTED APR 8 1975

3,876,512

FIG. 1



FIG. 2



## ELECTROLYTIC CARBURIZING PROCESS USING A CARBONATE ELECTROLYTE

The present invention relates to a carburizing process by electrolysis.

In the conventional carburizing process, melted salt of cyanide is widely used because such process is comparatively simple. However, this conventional process has disadvantages that cyanide is poisonous, the control of a bath is difficult and carburizing can not be prevented by electroplating steel with copper. The present invention eliminates the above disadvantages completely, above all it has a great advantage not to cause pollution.

### IN THE ACCOMPANYING DRAWING

FIG. 1 is a schematic illustration of electrolysis device used in the present invention; and

FIG. 2 shows the relation between current and carbon potential.

The process for carburizing according to the present invention will be explained with reference to the drawing. In the bath 4 of a furnace 1, an object article 2 to be carburized and a graphite electrode 3 are immersed. An electric power source 5 is connected between the object article and the graphite electrode through a variable resistor 6 and an ammeter 7. The reference numeral 8 designates a voltmeter and 9 indicates an electric heater. The principal component of the bath 4 is  $MCO_3$  ( $M$  is metal element), which metal element is melted by the electric heater. When principal component of the bath is  $Na_2CO_3$  as an example of  $MCO_3$  and the positive and negative poles of the DC or pulsating current power source 5 are respectively connected to the object article 2 to be carburized as the cathode and to the graphite electrode 3 as the anode, the following reaction takes place.

Reaction on the cathode side:



Where,  $e^-$  is Na electron, and  $CO_3^{2-}$  is decomposed into  $CO_2$  or  $CO$ .

$CO_2 + 4Na \text{ (nascent state)} = 2Na_2O + C \text{ (nascent state, perform carburizing)}$

$CO + 2Na \text{ (nascent state)} = Na_2O + C \text{ (nascent state, perform carburizing)}$

Reaction on the anode side:



$CO_3 + 2C = 3CO$  (Agitation occurs due to Peltier effect).

$CO_2 + C = 2CO$  (Agitation occurs due to Peltier effect).



Reaction on the surface of the bath:



As mentioned above, melted salt whose principal component is  $MCO_3$  is ionized to produce  $M$  of nascent state on the cathode side (on the side of the object article).  $M$  of nascent state reacts with  $CO_2$  or  $CO$  generated by the decomposition of  $CO_3$  to produce  $C$  which

performs carburizing. On the other hand,  $CO_3$  of nascent state produced on the anode side instantly produces  $CO_2$  or  $CO$  by pure chemical reaction. The resulting  $CO_2$  reacts with  $C$  to form  $CO$ .

5 Voltage higher than the sum of the electrolytic potential of  $CO_3^{2-}$  and overvoltage of the graphite electrode is applied to the anode.  $CO_2$  or  $CO$  thus produced diffuses toward the cathode rapidly by Peltier effect. Therefore, a complicated article such as a gear is uniformly carburized.

Further, in accordance with the present invention, decarburization can also be performed by controlling current. FIG. 2 shows the relationship between current and carbon potential at the cathode of an embodiment

15 of the present invention. When the current is  $0.01A/cm^2$  or less, the carbon potential becomes negative. Thus, at this low current, carbon atoms are removed from the cathode resulting in decarburization of the cathode, so that carburizing can be adjusted easily

20 by controlling the current. The above mentioned carburizing is a quite novel process. It is also possible to use a neutral salt by regulating current.

Another feature of the present invention is that sludge does not deposit on the bottom of the furnace 25 unlike the conventional carburizing process, promising long life of the bath, since the reaction to produce  $MCO_3$  takes place on the surface of the bath.

### EXAMPLE

30 An automobile transmission gear was carburized by the above mentioned process according to the present invention. Object article to be carburized: Automobile transmission gears of 77mm and 42mm in diameter, made of SMC21. Composition of the bath: 50 percent of  $Na_2CO_3$  + 150 percent of NaCl ( $Na_2CO_3$  alone will be effective, but NaCl was added to make carburizing easier at lower temperatures.)

|    |                   |               |
|----|-------------------|---------------|
| 40 | Voltage:          | 2V            |
|    | Current:          | $0.3 A/cm^2$  |
|    | Bath temperature: | $927^\circ C$ |
|    | Carburizing time: | 60 minutes    |
|    | Quenching:        | Oil           |

What is claimed is:

1. Carburizing process characterized by connecting an object article to be carburized as cathode and graphite as an anode in melted salt consisting of  $MCO_3$ , and electrolyzing the melted salt.

2. A process in accordance with claim 1 in which the melted salt is  $Na_2CO_3$ .

3. Carburizing process characterized by connecting an object article to be carburized as a cathode and graphite as an anode in melted salt consisting of  $MCO_3$  and NaCl, and electrolyzing the melted salt.

4. A process in accordance with claim 3 in which the melted salt consists of one part by weight of  $Na_2CO_3$  and three parts or less by weight of NaCl.

\* \* \* \*

UNITED STATES PATENT OFFICE  
CERTIFICATE OF CORRECTION

Patent No. 3,876,512 Dated April 8, 1975

Inventor(s) Hiyama, Shinji

It is certified that error appears in the above-identified patent and that said Letters Patent are hereby corrected as shown below:

Column 2, Line 16, after "potential" insert --at the cathode--.

In the Title Page, the following drawing should be shown in place of the figure illustrated.



Signed and Sealed this  
thirtieth Day of September 1975

(SEAL)

Attest:

RUTH C. MASON  
Attesting Officer

C. MARSHALL DANN  
Commissioner of Patents and Trademarks